

1

3,189,540  
PRODUCTION OF LUBRICATING OILS BY  
CATALYTIC HYDROGENATIONRobert H. Kozlowski, Berkeley, and Robert L. Jacobson,  
Pinole, Calif., assignors to California Research Corporation,  
San Francisco, Calif., a corporation of Delaware

No Drawing. Filed Jan. 2, 1962, Ser. No. 163,923

4 Claims. (Cl. 208—264)

This application is a continuation-in-part of copending application Serial No. 12,319, filed March 2, 1960, now U.S. Patent No. 3,114,701.

This invention relates to the production of lubricating oils by catalytic hydrogenation, and in particular the invention relates to the production of lubricating oils of improved color by catalytic hydrogenation of petroleum oils rich in polycyclic hydrocarbons and containing nitrogen compounds, using certain high metal content, sulfided, nickel-molybdenum-alumina catalysts. Still more particularly, the invention relates to an improved process using relatively severe conditions of catalytic hydrogenation controlled to remove a specified fraction of the nitrogen content of a petroleum oil and thereby to obtain a lubricating oil product of improved properties.

The use of catalytic hydrogenation in the refining of lubricating oils is well known. Mild hydro-finishing has been employed as a substitute for acid treating or clay contacting of refined lube oils, using relatively mild conditions of low temperature, low pressure, and high space velocity. Destructive hydrogenation has also been proposed as a substitute for solvent extraction of crude lube oils, using severe conditions of high temperature and pressure. The catalysts employed in the prior art processes are usually either hydrofining catalysts such as molybdenum oxide, cobalt, molybdate, nickel-tungsten sulfide, etc., or hydrogenation catalysts, such as nickel or platinum. Usually the catalyst metals, oxides, or sulfides, are supported on a carrier such as alumina, silica-alumina, or magnesia. The supported hydrofining catalysts have invariably a low metal content of less than 15% by weight.

We have found that certain high metal content sulfided nickel-molybdenum-alumina catalysts give outstanding results in the catalytic hydrogenation of petroleum oils rich in polycyclic hydrocarbons, particularly with respect to producing lube oils of improved color. Thus, for example, when a bright stock (187 SSU at 210° F.) was subjected to catalytic hydrogenation by contacting with a prior art hydrofining catalyst containing 2.8% cobalt and 6.7% molybdenum, on alumina, at 1000 p.s.i.g., 600° F., and 0.5 volume of oil per volume of catalyst per hour (LHSV), with 2000 s.c.f. of H<sub>2</sub> per barrel of oil, the ASTM color was improved from 8 to 6.5. When a sulfided 6% nickel-20% molybdenum, on alumina, catalyst was used at the same conditions, the ASTM color was improved from 8 to 5.5. At greater severity, for example, 650° F. and with other conditions comparable, product color improved even more, from 8.0 to 3.5, with the sulfided Ni-Mo catalyst. Similar superior results are obtained in the catalytic hydrogenation of distillate lube oils with the high metal content sulfided catalysts. Also, even better color is obtained at more severe conditions of elevated temperature and pressure and low space velocity.

The high metal content sulfided nickel-molybdenum-alumina catalysts used in the process of this invention contain 3-10% by weight nickel and 12-30% by weight molybdenum, with the more active catalysts containing 4-10% nickel and 15.5-30% molybdenum. The atomic ratio of nickel to molybdenum is in the range of 0.25 to 0.8, preferably about 0.6. A typical preferred catalyst will contain about 6 weight percent nickel and about 20 weight percent molybdenum. The catalysts may be prepared by alternate impregnation of a support consisting essentially of alumina, calcining after each impregnation

2

to convert the metal compounds to the metal oxides; or they may be prepared by simultaneous coprecipitation of aluminum, molybdenum, and nickel compounds; or by coprecipitation of aluminum and molybdenum compounds followed by impregnation with nickel, and with additional molybdenum, if desired. The catalysts are sulfided before use in the process. A special property of these catalysts when sulfided is their unusually high activity for the removal of nitrogen from petroleum oils containing nitrogen compounds by catalytic hydrogenation of the nitrogen compounds to ammonia. Thus, for example, the catalysts are found to be from two to five times as active as prior art hydrofining catalysts for the removal of nitrogen from neutral distillate lube oils. The catalysts, their preparation, and their use in processes for the substantially complete removal of nitrogen from distillable hydrocarbon oils are disclosed in our pending applications Serial Nos. 12,319, filed March 2, 1960, now U.S. Patent No. 3,114,701; 12,466, filed March 2, 1960, now abandoned; and 90,382, filed February 20, 1961, now abandoned.

In accordance with the catalytic hydrogenation process of this invention, a petroleum oil rich in polycyclic hydrocarbons and containing nitrogen compounds is hydrogenated by contacting with a high metal content, sulfided, nickel-molybdenum-alumina catalyst containing 3-10 weight percent nickel and 12-30 weight percent molybdenum, in the presence of excess hydrogen at a partial pressure of over 800 p.s.i.a., at 600-800° F., and 0.2-3 LHSV. The hydrogen partial pressure, temperature, and space velocity are controlled within the foregoing ranges to remove a specified fraction of the nitrogen content of the oil. When the conditions are so controlled, the degree, fraction or percent nitrogen removal from a petroleum oil is found to be a direct index of the degree of change in color and certain other properties of the oil which reflect the hydrogenation of unsaturated and unstable compounds therein. The lube oil properties found to be so related to the extent of hydrogenation in terms of nitrogen removal are expressed in somewhat arbitrary measurements, in particular: color, viscosity, pour point, oxidation stability, and additive response. Improvement to a desired extent of at least one lube oil property, in addition to color, selected from the group consisting of viscosity, pour point, oxidation stability, and additive response, is achieved by controlling the conditions to obtain from 30 to 60 percent nitrogen removal in the catalytic hydrogenation process of this invention.

Preferred lubricating oils are essentially naphthenic in basic structure, and have alkyl substituents of varying complexity. Essentially paraffinic or waxy hydrocarbons are not desired, nor are essentially aromatic hydrocarbons, because of their poor lubricating properties. Hence, the petroleum oils from which lubricating oils are produced by this invention are petroleum oils rich in polycyclic hydrocarbons, and which contain nitrogen compounds. Predominantly paraffinic petroleum oils are not suitable feed stocks for the process because such compounds are not converted to the desired naphthenes by the catalysts at the conditions used in the process. In general, the suitability of a petroleum oil as feed declines as the paraffin content increases. Preferred petroleum oil feeds are partially refined lube oil stocks, such as bright stocks, neutrals, and raffinates of naphthenic crude. Crude lube cuts from highly naphthenic crude petroleum are also suitable, however, though the hydrogenated product may require mild dewaxing.

The nitrogen content of petroleum oils rich in polycyclic hydrocarbons is present primarily as heterocyclic nitrogen compounds. Removal of the nitrogen improves the lube oil not only by eliminating the highly colored nitrogen compounds, but also by converting such het-

erocyclics to naphthenic lubricating oil hydrocarbons. Hence, the process of the invention not only purifies lube oils but also produces lube oils.

Since the high metal content, sulfided, nickel-molybdenum-alumina catalysts are unusually active for hydrogenation of nitrogen compounds, the conditions used in the process of this invention are peculiar to the catalysts. Although with these catalysts more moderate conditions of temperature, pressure, and space velocity could be employed to remove a specified fraction or percent of the nitrogen content of an oil, in general higher pressures, above 800 p.s.i., are employed in the invention, as compared to hydrofining processes of the prior art where only mild hydro-finishing was contemplated.

In carrying out the catalytic hydrogenation of this invention any suitable equipment arrangement may be used for contacting the oil with the catalyst in the presence of excess hydrogen. For example, the catalyst may be maintained as one or more fluidized beds, gravitational beds, or fixed beds of small particles, through which the oil and hydrogen are passed, upflow or downflow, concurrent or countercurrent. A slurry of catalyst in oil may also be used. Usually, the catalyst is in the form of small pellets or rod-like extrusions contained in a reactor as several fixed beds, and the oil and hydrogen are passed together downflow through the beds at controlled temperature, pressure, and flow rates. The effluent is cooled to separate product oil from hydrogen-rich gas, while is recycled. To maintain a high hydrogen partial pressure and to insure that excess hydrogen is present, the hydrogen-to-oil ratio is from 1,000 to 10,000 or more standard cubic feet per barrel (s.c.f./bbl.), usually 2,000-6,000 s.c.f./bbl.

The total pressure depends on the purity of the hydrogen supplied and whether and under what conditions hydrogen is recycled. The hydrogen partial pressure is above about 800 p.s.i.a., and may range upwards of 10,000 p.s.i.a. Pressures of 1,000-3,000 p.s.i.a. are preferred. At such pressures color improvement is accomplished over a broad range of temperatures, from 600° F. to 800° F., permitting maximum flexibility in control of the nitrogen removal. Preferred temperatures are between 600 and 750° F. for the limited nitrogen removal desired in this invention, especially temperatures of 650-700° F. Space velocities of 0.2-3 LHSV are used, preferably 0.5-2 LHSV, to obtain the technical and economic advantages of adequate contacting time in equipment of reasonable dimensions. At milder conditions of lower pressure, i.e., below 800 p.s.i., nitrogen removal is a less reliable index of the degree of hydrogenation of the oil, the advantages gained by using the high metal content, sulfided, nickel-molybdenum-alumina catalysts are less pronounced, and the range of temperatures at which color improvement is obtained is narrower.

The new concept of this invention, the method of using it, and the advantages obtained thereby may be best explained and understood by means of examples. In the following examples, where reference is made to a

sulfided nickel-molybdenum catalyst, the catalyst employed was prepared by impregnating a high purity alumina base with nickel nitrate, calcining, then impregnating with ammonium molybdate, and calcining, again impregnating with ammonium molybdate, and calcining. The oxide catalyst, which contained 6% nickel and 20% molybdenum, was sulfided by contacting with hydrogen containing dimethyl-disulfide, equivalent on hydrogenation to 2% H<sub>2</sub>S, at about 500° F. to convert the metal oxides substantially to the sulfides prior to use in the catalytic hydrogenation process. The first example illustrates an embodiment of the invention in the production of low cold test lubricating oil of improved color and oxidation stability from a naphthenic crude by a combination of mild solvent extraction followed by catalytic hydrogenation at controlled conditions.

#### EXAMPLE I

A naphthenic California crude was distilled to obtain a heavy crude lube distillate amounting to about 8 volume percent of the crude, and boiling from about 500° F. to about 700° F. at 10 mm. Hg. The distillate was solvent treated by phenol extraction at varying solvent-to-oil ratios to obtain lube oil raffinates at volumetric yields of 40%, 60%, and 70%. Properties of the raffinates are listed in Table I. The 40% yield raffinate represents low cold test lube oil produced by the prior art without catalytic hydrogenation. The 60% and 70% raffinates are of poor quality with respect to color and oxidation stability, and have higher than the desired viscosity. The 60% and 70% raffinates were then subjected to catalytic hydrogenation by contacting with the sulfided nickel-molybdenum catalyst at conditions controlled to remove different fractions of the nitrogen content. The treating conditions used and the product properties obtained are listed in Table II.

Table I

| Property                             | Desired product  | Raffinate yield |       |       |
|--------------------------------------|------------------|-----------------|-------|-------|
|                                      |                  | 40%             | 60%   | 70%   |
| Gravity, °API                        |                  | 21.7            | 19.9  | 19.3  |
| Viscosity, SSU at 100° F.            |                  | 1,638           | 2,525 | 2,879 |
| Viscosity, SSU at 210° F.            | 85-95            | 86.3            | 97    | 101   |
| Color, ASTM                          | Less than 4.5    | 4               | 5     | 6.5   |
| Pour point, °F.                      | Less than +10    | -10             | -     | +5    |
| Natural oxidation stability, hours   | Greater than 7   | 12              | 4.9   | 3.6   |
| Catalyzed oxidation stability, hours | Greater than 1.8 | 1.9             | 0.8   | 0.8   |
| Nitrogen, p.p.m.                     |                  | 800             | 1,660 | 2,400 |
| Aromatics, percent                   |                  | 9               | 14    | 15.5  |

NOTE.—Natural oxidation stability is the time required for a given volume of the oil, as is, to absorb one liter of oxygen from air bubbled through the oil at a temperature controlled at 340° F. Catalyzed oxidation stability is the time required for the oil to absorb one liter of oxygen at the same conditions when 3.7 weight percent of a commercial oxidation inhibitor (Oronite lube oil additive 2306) is added and the oxidation is catalyzed by added iron and copper impurities. This property is a measure of the additive response of the lube oil, as the amount of metal oxidation catalyst added would be sufficient to cause virtually immediate discoloration of the oil in the absence of an oxidation inhibitor. Aromatics was determined by the n-d-M method, and is expressed in percent of carbon atoms present in aromatic rings.

Table II

| Feed treated                          | 60% Raffinate |       |       |       | 70% Raffinate |       |       |       |
|---------------------------------------|---------------|-------|-------|-------|---------------|-------|-------|-------|
|                                       | 2,000         | 1,990 | 2,020 | 2,020 | 1,980         | 2,000 | 2,000 | 1,980 |
| Conditions:                           |               |       |       |       |               |       |       |       |
| Pressure, p.s.i.a. H <sub>2</sub>     | 2,000         | 1,990 | 2,020 | 2,020 | 1,980         | 2,000 | 2,000 | 1,980 |
| Temperature, °F.                      | 550           | 600   | 640   | 695   | 600           | 650   | 675   | 700   |
| Space velocity, LHSV                  | 1.25          | 1.25  | 1.14  | 1.18  | 1.35          | 1.48  | 1.48  | 1.40  |
| Gas rate, s.c.i. H <sub>2</sub> /bbl. | 5,100         | 4,800 | 4,800 | 6,000 | 4,800         | 4,500 | 4,100 | 4,600 |
| Product properties:                   |               |       |       |       |               |       |       |       |
| Gravity, °API                         | 20.8          | 21.5  | 22.3  | 22.7  | 20.7          | 21    | 21.1  | 22.4  |
| Viscosity, SSU at 100° F.             | 2,227         | 1,973 | 1,759 | 1,351 | 2,173         | 1,918 | 1,713 | 1,436 |
| Viscosity, SSU at 210° F.             | 92.8          | 89    | 85.3  | 77.6  | 91            | 86.8  | 83.3  | 78.4  |
| Color, ASTM                           | 2             | 1.5   | 1     | 1     | 1.5           | 1.5   | 1.5   | 1.5   |
| Pour point, °F.                       | 0             | 0     | -5    | -10   | -5            | 0     | -5    | -5    |
| Natural oxidation stability, hours    | 6.2           | 7.6   | 11.5  | 0.7   | 6.8           | 9.4   | 15.1  | 3.8   |
| Catalyzed oxidation stability, hours  | 1.1           | 1.2   | 1.8   | 2.8   | 1.3           | 1.2   | 1.7   | 2.5   |
| Nitrogen, p.p.m.                      | 1,655         | 1,630 | 1,100 | 615   | 2,100         | 1,530 | 1,240 | 905   |
| Aromatics, percent                    | 13            | 12    | 10    | 7.5   | 12.5          | 10    | 10    | 10.5  |
| Percent nitrogen removal              |               |       | 32    | 62    | 12.5          | 36    | 48.3  | 62.5  |

The catalytic hydrogenation of Example I improved the color in every case and improved the oxidation stability of the raffinates to the desired extent when the operating conditions were controlled to remove 30-60% of the nitrogen content, with an optimum apparently at about 40-50% removal. The viscosity, however, dropped more than would be desired. In a novel embodiment of the present invention, product lube oil of the desired viscosity is produced at greater over-all yield by starting with a crude lube distillate of higher than the desired boiling range, solvent treating the distillate to obtain a high yield of raffinate of higher than the desired viscosity and of poor quality with respect to color and oxidation stability, and then subjecting the raffinate to catalytic hydrogenation by contact with a high metal content, sulfided, nickel-molybdenum catalyst at conditions of temperature, hydrogen partial pressure, and space velocity controlled in the ranges 650-750° F., at least 1500 p.s.i.a., and 0.5-3 LHSV, to remove 30-60% of the nitrogen content and thereby to adjust the color, viscosity, and oxidation stability to the desired values. That an increased yield of superior product is obtained thereby is illustrated by the following example.

#### EXAMPLE II

The naphthenic crude of Example I was distilled to obtain a broader lube oil distillate amounting to about 9 volume percent of the crude by including higher boiling material. The distillate was solvent treated by phenol extraction to obtain a poor quality lube oil raffinate at 60% yield. The raffinate was then subjected to catalytic hydrogenation by contacting with the nickel-molybdenum catalyst at 2000 p.s.i.a. hydrogen partial pressure, 675° F., and 1.3 LHSV, with 6700 s.c.f. of H<sub>2</sub> per barrel. Properties of the raffinate feed and the lube oil product are given in Table III. Processing in this way increases the yield of product lube oil from crude by 47.5% as compared to the solvent treating method formerly used.

Table III

| Property                             | Raffinate | Product |
|--------------------------------------|-----------|---------|
| Gravity, ° API                       | 20.2      | 22.5    |
| Viscosity, SSU at 100° F.            | 2,774     | 1,715   |
| Viscosity, SSU at 210° F.            | 103.6     | 86.3    |
| Color, ASTM                          | 8         | 1.5     |
| Pour point, ° F                      | 0         | 0       |
| Natural oxidation stability, hours   | 4.6       | 12.5    |
| Catalyzed oxidation stability, hours | 0.8       | 2.1     |
| Nitrogen, p.p.m.                     | 1,710     | 1,050   |
| Aromatics, percent                   | 13.5      | 39      |
| Percent nitrogen removal             |           |         |

The conditions of temperature, pressure, and space velocity may be altered within limits to obtain the same fraction of nitrogen removal and thereby to obtain the same improved product. However, for the treatment of raffinates, the pressure should be relatively high, i.e., above 1500 p.s.i.a. H<sub>2</sub>, preferably at least 2000 p.s.i.a. Lower temperatures may be used at lower space velocities, but we prefer for the best results to use a space velocity of at least 0.8. The temperature can then be in the preferred range of 650-750° F. Ordinarily, the temperature is increased over a period of time to compensate for catalyst deactivation. However, the conditions of Example II were maintained for over 1000 hours without any noticeable deactivation or catalyst fouling by coke deposits.

The invention may also be used to produce residual or non-distillate lube oils of improved color and oxidation stability, for example, bright stock. A high natural oxidation stability is a valuable property of bright stock because such oils are used to a great extent in compounded lubricants. The present invention produces bright stock of improved color and having maximum oxidation stability by catalytic hydrogenation of nitrogen-containing bright stock at conditions controlled with

in the ranges 800-2000 p.s.i.a. hydrogen partial pressure, 600-700° F., and 0.5-3 LHSV, to remove 20-60% of the nitrogen content. This is illustrated by the following example.

#### EXAMPLE III

A bright stock boiling entirely above 300° F. at one millimeter mercury absolute pressure was contacted with the sulfided nickel-molybdenum catalyst at 1000 p.s.i.a. H<sub>2</sub>, 650° F., 0.5 LHSV, and 6000 s.c.f. H<sub>2</sub> bbl. Properties of the feed and product are given in Table IV.

Table IV

| Property                             | Feed  | Product |
|--------------------------------------|-------|---------|
| Gravity, ° API                       | 24.8  | 25.6    |
| Viscosity at 100° F.                 | 4,055 | 3,119   |
| Viscosity at 210° F.                 | 190.8 | 168.3   |
| Viscosity index                      | 89    | 93      |
| Color, ASTM                          | 8     | 3.5     |
| Natural oxidation stability, hours   | 8.7   | 17      |
| Catalyzed oxidation stability, hours | 2.7   | 3.1     |
| Nitrogen, p.p.m.                     | 800   | 375     |
| Percent nitrogen removal             |       | 53      |

Similar results were obtained by catalytic hydrogenation at 1000 p.s.i.a., 700° F., and 2.4 LHSV. At more severe conditions the oxidation stability is adversely affected; at mild conditions the oxidation stability is not improved.

As shown, the invention can also be used to improve the additive response of bright stock, for example, to oxidation inhibitors. This is of particular value where the bright stock is to be used in compounded lubricating oils such as high viscosity turbine oils.

A turbine oil comprising 40% bright stock was prepared using the product of Example III. With 0.25 weight percent of a commercial oxidation inhibitor added, the turbine oil had a life of 2,140 hours in a turbine oil standard test.

From the foregoing, it is seen that the exact conditions of temperature, pressure, and space velocity to be employed in a particular case depend on the properties of the particular feed stock and the properties of the lube oil desired. Thus, for example, in the case of two petroleum oils of similar boiling range but different nitrogen contents, the oil of higher nitrogen content will require somewhat more severe conditions to accomplish the same percent removal of nitrogen as the lower nitrogen content stock. However, these somewhat more severe conditions are found to be required also to obtain the desired improvement in the lube oil properties. This is illustrated by a comparison of the similar feeds of Examples I and II. Thus, with the particular objective of this invention in mind, and having the examples herein before him, one skilled in the art will, with but minimal experimentation to verify the estimates, be able with reasonable accuracy to predict the appropriate conditions to use with the sulfided nickel-molybdenum catalysts to obtain a desired lube oil product. Hence, the examples themselves are not to be considered limiting, and the true scope of the invention is defined by the following claims.

60 We claim:

1. A process for producing lubricating oil of improved color and natural oxidation stability which comprises solvent refining a heavy petroleum oil to obtain a solvent-refined lubricating oil fraction rich in polycyclic hydrocarbons, containing heterocyclic nitrogen compounds and having poor color above 4.5 on the ASTM scale and poor natural oxidation stability, hydrogenating said solvent refined fraction by contacting in the presence of excess hydrogen with a sulfided nickel-molybdenum-alumina catalyst containing between 4 and 10 weight percent nickel and between 12 and 30 weight percent molybdenum at reaction conditions in the ranges 800-3000 p.s.i.a. hydrogen partial pressure, 600-750° F., and 0.2-3 LHSV, while controlling the reaction conditions in a narrow range

within said ranges appropriate for the particular solvent-refined fraction to obtain only partial removal amounting to between 30% and 60% of the nitrogen from said oil,

and recovering as the product hydrogenated lubricating oil having improved color below 4.5 on the ASTM scale and improved natural oxidation stability.

2. The process of claim 1 wherein said heavy petroleum oil is a residual petroleum oil, which is solvent refined to obtain as said solvent-refined lubricating oil fraction a bright stock, and the reaction conditions are controlled during contacting said bright stock with said sulfided catalyst within the ranges 800-2000 p.s.i.a. hydrogen partial pressure, 600-700° F., and 0.5-3 LHSV.

3. A process in accordance with claim 1 wherein said heavy petroleum oil is a heavy vacuum distillate of naphthenic crude petroleum from which distillate there is recoverable by phenol extraction a raffinate of desired viscosity having acceptable color and oxidation stability only if limited to a raffinate yield of less than 50% by virtue of said distillate having a higher average boiling point than desired for said raffinate, which comprises carrying out the solvent refining of said distillate to obtain as said solvent-refined lubricating oil fraction a raffinate of poor color and oxidation stability in greater than 50% yield and having higher than desired viscosity, controlling the reaction conditions during said hydrogenating in the ranges 1500-3000 p.s.i.a. hydrogen partial pressure, 650-750° F., and 0.5-3 LHSV, and recovering as said product

low cold test lubricating oil of the desired viscosity having improved color and oxidation stability in a greater yield than is obtainable from the naphthenic crude by distillation and extraction.

4. The process of claim 3 wherein the reaction conditions during said hydrogenating are controlled in the ranges 2000-3000 p.s.i.g., 650-750° F., and 0.8-3 LHSV to limit the removal of nitrogen compounds to between 40% and 50%, and there is recovered as the product low cold test lubricating oil having a color below 4 on the ASTM scale and a natural oxidation stability greater than 7 hours.

References Cited by the Examiner

UNITED STATES PATENTS

|           |       |                 |         |
|-----------|-------|-----------------|---------|
| 2,706,167 | 4/55  | Harper et al.   | 208-264 |
| 2,905,625 | 9/59  | Berger          | 208-254 |
| 2,905,636 | 9/59  | Watkins et al.  | 208-254 |
| 2,944,006 | 7/60  | Scott           | 208-89  |
| 2,983,676 | 5/61  | Howland         | 208-254 |
| 2,988,501 | 6/61  | Inwood          | 208-254 |
| 3,004,913 | 10/61 | Tucker          | 208-544 |
| 3,014,860 | 12/61 | Douwes et al.   | 208-254 |
| 3,046,218 | 7/62  | Henke et al.    | 208-144 |
| 3,094,480 | 6/63  | Richardson      | 208-143 |
| 3,105,813 | 10/63 | Gutberlet       | 208-254 |
| 3,114,701 | 12/63 | Jacobson et al. | 208-254 |

ALPHONSO D. SULLIVAN, Primary Examiner.

UNITED STATES PATENT OFFICE  
CERTIFICATE OF CORRECTION

Patent No. 3,189,540

June 15, 1965

Robert H. Kozlowski et al.

It is hereby certified that error appears in the above numbered patent requiring correction and that the said Letters Patent should read as corrected below.

Column 1, line 17, for "alumnia" read -- alumina --; column 3, line 30, for "while" read -- which --; column 6, line 37, after "test." insert -- With normal bright stock the life is 940 hours. --.

Signed and sealed this 7th day of December 1965.

(SEAL)

Attest:

ERNEST W. SWIDER  
Attesting Officer

EDWARD J. BRENNER  
Commissioner of Patents